

## UNITED STATES PATENT OFFICE

1,942,041

## ALLOY

Robert T. Wood, Cleveland, Ohio, assignor, by  
mesne assignments, to Magnesium Develop-  
ment Corporation, a corporation of Delaware

No Drawing. Application November 17, 1932  
Serial No. 643,033

2 Claims. (Cl. 75—1)

The invention relates to magnesium base alloys and is directed to the development of alloys of this class which, while possessing the desirable characteristics of the class as a whole, are further characterized by increased tensile strength and high yield point, as well as by a greatly increased elongation.

The use of magnesium base alloys has been quite seriously limited by a number of considerations such as difficulty of working and casting, and inferior tensile strength as compared with many of the strong aluminum alloys. It is quite generally appreciated that any improvement in magnesium alloys which means increased yield point, strength and elongation will be very valuable, and for this reason efforts have been continuously expended in the search for improvement along these lines. It is to this general object that the present invention is directed.

A particular object of the invention is the modification of magnesium base alloys containing tin and manganese, by the addition thereto of aluminum as a principal alloying ingredients with or without the addition of lesser amounts of zinc, to produce an alloy of increased tensile strength, yield point and elongation.

I have discovered a very useful range of composition over which aluminum additions are particularly effective in producing the desired improvement in tensile properties without serious detriment to the other properties of this class of alloys. According to my invention, the alloys may contain from 0.1 to 12.0 per cent of tin, from 0.5 to 6.0 per cent of aluminum, and from 0.1 to 1.0 per cent of manganese. The aluminum increases the tensile strength as much as 15 per cent, the yield point as much as 20 per cent, and the elongation as much as 100 per cent. As a result of the tests which I have conducted, I have found further that the magnesium alloy containing tin, aluminum and manganese is superior to a magnesium base alloy containing only aluminum because of improved hot-working characteristics, particularly hammer-forging characteristics. The alloy can also be extruded.

The improvement in physical properties is particularly marked throughout what I consider to be the preferred range of composition, which includes alloys containing from 4.0 to 6.0 per cent of tin, 3.5 to 4.5 per cent of aluminum, and 0.5 to 0.8 per cent of manganese. As an example of my preferred composition, I have produced an alloy containing 5.6 per cent of tin, 4.2 per cent of aluminum, and 0.8 per cent of manganese. Tests performed on this alloy in the unheat-treated and hammer-forged condition showed the alloy to have a tensile strength of 37,500 pounds

per square inch, a yield point of 21,000 pounds per square inch, and an elongation of 12.0 per cent in two inches as compared with the properties 60 of a similar alloy not containing aluminum which had a tensile strength of 33,000 pounds per square inch, a yield point of 17,000 pounds per square inch, and an elongation of 6.5 per cent in two inches. This comparison shows an unusual property of my alloys, which is the fact that tensile strength and elongation are simultaneously increased.

When my improved alloys are used for extrusion purposes they may also contain zinc in 70 amounts ranging from 0.1 per cent to 5 per cent. The addition of zinc in the amounts indicated gives superior properties to the alloy in the extruded condition and the improvement is particularly manifested when the zinc is present in 75 amounts of from 1 to 3 per cent. The addition of zinc is likewise generally beneficial to my improved alloys, but if the alloys are to be forged or rolled, as distinguished from extruded, the alloys should preferably not contain over about 80 1 per cent of zinc.

I have found that tin increases the corrosion resistance of the magnesium base aluminum-zinc-manganese alloys without adversely affecting the mechanical properties. The results of 85 the tests which I have conducted indicate that the increase in corrosion resistance is quite noticeable when the alloy is in the extruded condition. While the magnesium base alloys containing tin, aluminum and manganese, with or without zinc, are entirely satisfactory in achieving 90 the objects and advantages hereinabove enumerated, other elements may be added to produce a new property in the alloys or to affect or modify an old property without substantially departing 95 from the invention so long as the material properties of the alloys are not substantially impaired.

The alloys herein disclosed and claimed may be subjected to the usual thermal treatments for 100 the purpose of improving or altering their properties.

I claim:

1. An alloy containing about 0.1 to about 12.0 per cent of tin, about 0.5 to about 6.0 per cent of aluminum, and about 0.1 to about 1.0 per cent of manganese, the balance being substantially magnesium.
2. An alloy containing about 4.0 to about 6.0 per cent of tin, about 3.5 to about 4.5 per cent 110 of aluminum, and about 0.5 to about 0.8 per cent of manganese, the balance being substantially magnesium.

ROBERT T. WOOD.